

## UNITED STATES PATENT OFFICE

2,228,976

MOLDING MATERIAL AND METHOD OF  
PRODUCING THE SAME

Herman J. Reboulet, Melrose, Mass., assignor to  
The Mead Corporation, Chillicothe, Ohio, a corporation of Ohio

No Drawing. Application July 11, 1936,  
Serial No. 90,265

4 Claims. (Cl. 260—124)

This invention relates to the recovery of materials from the spent digestion liquors in the paper industry, and more particularly to materials usable in the production of molded articles and methods for effecting the recovery and for producing the moldable materials.

One of the principal objects of the invention is to provide a method adapted for the treatment of spent digestion liquors resulting in the chemical digestion of fibrous materials to produce pulp in the paper industry to produce therefrom a recovered lignin material which is moldable in itself, and which lends itself to effective intermixiture with other moldable and filler materials to provide molded products of superior commercial characteristics.

Another object is to produce such an organic recovered material.

It is a further object to provide a process for the recovery of such non-cellulosic material which process is coordinated with the usual recovery system in the paper making plant in a highly economical manner.

Other objects and advantages will be apparent from the specification and the appended claims.

As is well known, it has been the practice for many years to produce most pulp for the manufacture of paper, and like products from materials such as wood, straw and the like by subjecting such fibrous material to so-called chemical digestion,—the fibrous material generally being immersed in the chosen digestion liquid and cooked under proper conditions of temperature, pressure, etc. While there are several well known forms of cook, the best known forms are the so-called sulfite, sulfate or kraft and soda,—the names being indicative of the characteristics of the chemicals forming the main digestive portion of the cooking liquor. Generally speaking the process is the same; but the resulting spent digestion liquor, in each of the several forms of cook, will contain chemical compounds which are dependent upon the character of the digesting chemicals in the original cooking liquor. In all of these digestions the chemical present reacts with part of the natural materials of the wood to remove the so-called lignins, pentosans and other non-cellulosic material, along with some portions of the cellulosic material, which are most readily affected by the chemicals, leaving the cellulose fibers freed of the bonding and adhering materials which bind them together to give the rigid character and form to the wood or other material which is being treated. It is this spent digestion liquor,

generally known as "black liquor," which is treated in the practicing of this invention.

As clearly explaining the invention in its preferred embodiment, reference is made herein-after, unless otherwise specified, to that black liquor which results in the so-called soda cook. In that cook the wood is immersed in a solution of a caustic soda, the proportions of which are well known in conventional practice, and the material is subjected to cooking therein until the non-cellulosic materials have been removed to give the desired resulting release of the cellulose fibers and fiber bundles. This black liquor from the soda process is strongly alkaline, even though the cook reactions have been completed. It has been found that if this alkaline soda liquor is subjected to a controlled neutralizing effect, with an acid such as carbonic acid, obtained by passing  $\text{CO}_2$  through the liquor, and the pH value controlled within proper range, certain organic materials which are non-cellulosic in character and which are believed to be derived from the material of lignin origin which is found in the black liquor will be separated out which have peculiar characteristics as to fusibility, susceptibility to hydrolizing, moldability and admixture with other materials, either filler or thermosetting molding materials, to give desired and superior molded products.

When  $\text{CO}_2$  is bubbled through such black soda liquor to effect the neutralizing action lignous derivative material is precipitated out of solution, the character of the lignous derivative compounds being contingent upon the pH value as established by this acid. And the quantity of such lignous derivative material which is precipitated out, and it is believed also its molecular construction, is believed directly dependent upon the pH value established, which in turn is dependent upon the hydrogen ion concentration of the neutralizing acid used. These lignin derivative material organic compounds are of indeterminate molecular construction, the original lignin itself being probably a mixture of complex organic molecules, and the lignin derivative material which is separated out by the neutralizing action is likewise a mixture of complex molecules of character so far not definitely determined. However, the pH value which is dependent upon the particular acid used and its hydrogen ion concentration, will determine the character of lignin derivative molecules precipitated out, generally speaking the higher the hydrogen ion content the higher the molecular weight of the lignin derivative material which is precipitated out. It is believed,

therefore, that in the practicing of this process the molecular construction of the lignin derivative material can be controlled by the proper selection of acid, as to its hydrogen ion concentration, and the resulting pH value, on the acid side, will be substantially a constant for any particular acid that might be used, within any normal range of concentrations that could be used in actual commercial practices. It has been discovered, therefore, that by proper selection of the neutralizing acid lignin derivative material of a particular molecular weight range can be precipitated out, and those materials of a molecular weight corresponding to some substantially different hydrogen ion content acid will not be formed, or at least in any controlling quantity, and therefore the final characteristics of a lignin derivative material may be determined and controlled by the selection of the neutralizing acid to give a properly controlling pH value within the solution as the lignin derivative material is being precipitated therefrom.

Furthermore it has been found that as the acid neutralizing agent is chosen so as to produce lignin derivative material which constitutes a predetermined separated proportion with respect to the original material available, that particular material will have characteristics as to moldability, etc., which are contingent upon or proportional to the relative amount of material removed. Therefore, by so controlling the pH value and the precipitating effect that a given proportion of lignin derivative material is obtained from a predetermined amount of black liquor, the constituents and the characteristics of the resulting derivative material may be controlled according to predetermined desired values.

Very satisfactory results in utilizing the above for the production of such lignin derivative material from black liquor have been secured, using the digestion or black liquor from the soda pulp process. Preferably the process is carried out using a black liquor which has been suitably concentrated to contain a greater proportion of solids than in its initially produced state, but not in such concentrated condition as to interfere with proper separation of the lignin material therein. In operations on a plant scale, very satisfactory results have been secured using a black liquor in which the solids had been increased to about 16% to 17%, the desired concentration of liquor being conveniently secured by blending suitable quantities of the liquor from different stages of the evaporators. With such black liquor the desired controlled results may be secured through the utilization of carbon dioxide gas to effect the neutralizing action. This gas when bubbled through the black liquor, at room temperatures, will reduce the alkalinity to a narrow pH value range between pH 7.8 and pH 9, this range normally lying between pH 7.9 and pH 8.5. It is found that as the pH values decrease, it becomes more difficult to absorb additional CO<sub>2</sub> into the liquor. Also on a plant scale the stack gas available contains a diluted CO<sub>2</sub> gas and for these reasons the pH value may suitably be carried down to about pH 8.3. In some cases the liquor has a tendency to foam as the CO<sub>2</sub> is passed therethrough. Such foaming may usually be controlled by the action of a stirring member operating vigorously in the layer of foam and in the topmost zone of the liquid. An antifoaming agent such as Turkey red oil or the like, may be added in small quantity, a fraction of a percent, and will further tend to prevent objectionable

foaming. With the alkalinity reduced to this pH value it is found that precipitation of lignin derivative material from the black liquor, in proportion of approximately 25% of the original solids in the black liquor, will result, and this lignin derivative material is of such chemical, etc., characteristics, that it will function very satisfactorily, in a superior manner and provide for obtaining products not heretofore known. The precipitated material is quite fine and remains in suspension. 10

To facilitate subsequent filtration the suspended non-cellulosic matter is subjected, either simultaneously or subsequently, to a coagulating action, preferably by heating the suspension to a predetermined temperature range. While the 15 non-cellulosic matter can be separated from the liquor with difficulty in the absence of heating as a coagulating step, a heating to a temperature range of the order of 50° C. to 80° or 90° C. is found to greatly assist in the filtration and to 20 shorten the time required. A heating materially beyond the range specified is undesirable as it tends to effect the formation of a gummy mass very difficult to filter and to handle. It appears however that a higher coagulating temperature 25 may be used when more effective agitation is secured. The liquor is heated preferably by means of a steam coil and is also preferably agitated simultaneously with the heating to assure uniformity of temperature throughout. 30

Prior to filtration, it is desirable to cool the liquor to substantially room temperature, as it is found that the filtration of the liquor while hot is difficult and results in a product of undesirable characteristics. The liquor may be cooled by 35 running a cooling fluid through the coils and is preferably simultaneously agitated by mechanical means or by the introduction of air jets or the like.

Following the cooling the liquor is filtered on a 40 suitable filter press and the filtrate, containing the larger part of the digestion chemicals, is pumped back to the evaporators of the usual recovery system. The precipitate on the filter is then preferably washed with water to remove soluble compounds from the non-cellulosic matter, such compounds including the remainder of the treating chemicals, such as sodium compounds in the case of the soda process, and the soluble organic compounds such as alkali metal salts of 45 organic acids. The wash water may also be returned to the usual recovery system inasmuch as it contains a certain quantity of the treating chemicals which it is desirable to recover. 50

The precipitated matter at this stage of the 55 processing is a thick colloidal suspension, similar to a gel and in this form there is still retained in occluded form a relatively material quantity of the black liquor which it is difficult to filter out by any ordinary filtering process. This liquor 60 may contain caustic and also organo-metallic compounds which are undesirable as deleteriously affecting the molding and fusing characteristics of the lignin product.

Accordingly the precipitated matter is then 65 treated with a strong acid, such as sulfuric acid, in an amount slightly in excess of that required for neutralization. Being an electrolyte, the acid breaks up the agglomerated gel formation, facilitating filtering. And remaining traces of caustic 70 are neutralized and the objectionable organo-metallic compounds are broken down. It is also found that such acid treatment improves the resistance of the material to hydrolysis and tends to produce a material having a lower fusion point. 75

both of these characteristics being more particularly important when the material is to be used in molding, for example. Only a limited amount of sulfuric acid is required, and consequently the cost of acid used in the process, and the problem of disposing of salts such as sodium sulfate, are greatly reduced.

The neutralized precipitate is then washed to remove acid, and any soluble salts and the washed material may be then dried either at room temperature or more rapidly in a drier at a suitable temperature below its fusion point, for example, at 150° C. and is then broken up or pulverized in any desired manner.

15 As a specific example of the carrying out of the invention, the following is given. The black liquor from the soda process, specific gravity approximately 1.12 and pH value of 11 to 12, is pumped into a wooden treater tank, equipped with 20 a spider type gas inlet. The black liquor is treated with purified stack gas, from a stack gas recovery system, for approximately 24 hours at which time it had a pH value of 8. It is then pumped into a wooden coagulating tank equipped 25 with heating and cooling coils and a similar gas inlet. The liquor is heated to 60° C. by means of the steam heating coil, and is then cooled by running water through the cooling coil. The heating operation requires several hours while the 30 cooling operation extends over a somewhat longer period, the contents of the tank being continuously agitated during the whole time. The liquor is then pumped into a wooden reservoir tank equipped with agitating means. From the reservoir 35 tank the liquor is pumped at a pressure of 5 lbs. per square inch into the filter press, which preferably is a lead lined Sweetland filter. The filtrate is pumped back to the evaporator and carried through the usual recovery system in the 40 paper mill plant.

Wash water is then pumped through the filter to wash out the soluble compounds, this wash water also being returned to the recovery system. Tests have shown that the wash water should be 45 added in approximately the ratio of 3000 gallons to 2000 gallons of black liquor of the character above described, such method resulting in a total recovery of approximately 98% of the caustic present in the black liquor. Thereafter 500 gallons of water containing 20 pounds of sulfuric acid, representing a small excess of acid, is pumped through the filter and recirculated for approximately 10 minutes and then drained off. The precipitated material is again washed with 55 3000 gallons of water to wash out the acid and remaining soluble salts. If it is not desired to run the first or alkaline wash water through the recovery system, the whole or a part thereof may be run into the second or acid wash water 60 and the neutralized wash water then run into the sewer. The washed material is then removed from the filter press, dried on a drum dryer and pulverized in a Raymond pulverizer. A material produced in this manner is found to have a fusion temperature of the order of 180° C. to 200° C. Furthermore the lignin product as so produced is 65 of such characteristics that its melting or fusing temperature is subject to control, in a manner to provide melting temperatures reduced below the value mentioned, if desired. Thus a lignin material can be produced having melting point characteristics within the range of conventional phenol formaldehyde resins, such as to be directly mixable and fusible therewith. For example, lignin produced in accordance with the pres-

ent method may have controlled melting point characteristics imparted to it of approximately 90° to 100° C. Reference is made to copending application Serial No. 29,168 filed June 29, 1935, for disclosure of the method of thus obtaining 5 controlled melting point characteristics.

It is found that the material so produced is very low in ash and in organo-metallic compounds, the ash content of several runs falling within a range of .03% to .10% ash. The above 10 results were obtained by using distilled water for washing, and somewhat larger ash contents are obtained when a relatively hard water is used, the ash in the latter case running up to approximately 1% ash. For most uses, however, it is 15 found that the higher ash content does not produce objectionable results where the ash results from materials present in hard water and consequently the use of hard water is a commercially practicable method of carrying out the invention. 20

The product of this invention, besides being relatively pure and substantially ash free, is homogeneous, is water insoluble in high degree, is acid resistant, is resistant to such solvents as benzol, carbon tetrachloride, and ether, and is found 25 to have very desirable characteristics for use as a binder material in molding, fuel briquetting, and the like. It also has the desirable property for some purposes of high solubility in diethylene oxide, phenols, pyrogallol, benzaldehyde aldol, 30 diethylene glycol monoethyl ether, and is also largely soluble in acetone, alcohol, and mixtures thereof. The process is extremely simple, makes use of inexpensive materials, and is so coordinated with the usual recovery process in the paper making plant that it provides for the carrying out 35 of the present invention in conjunction with the usual recovery system for the recovery of caustic as in the said process.

When this material is mixed with a filler such 40 as wood flour, asbestos, carbon black, or kieselguhr, and hot pressed in a mold, it serves as a highly effective binder and the resulting molding material has very desirable properties. It is readily fusible, has thermoplastic properties, and 45 can be repeatedly cooled and reheated without obtaining a permanent set. When this material is used in excess of 30% by weight of the molding composition, the product is found to have good strength and low water absorption characteristics. Furthermore, it is resistant to sulfuric acid, 50 solvents such as naphtha and benzol, and lubricating oil.

The material of this invention can be satisfactorily molded over a wide range of temperatures 55 and pressures but the molding is preferably carried out under conditions of the order of those of standard practice. Thus for instance, a mixture of between 30% to 80% of the binder of this invention, and 70% to 20% filler can be molded 60 with very satisfactory results at temperatures of the order of 175° C. and pressures of the order of 1100 lbs. per square inch, with a molding time of two minutes. The product being thermoplastic, it is placed in the mold and subjected to heat 65 and pressure, the mold then being allowed to cool while the pressure is maintained.

The binder material of this invention can be used as a substitute for all or a part of known 70 thermoplastic binders in molding compositions, an example of such known thermoplastic binder being shellac. As an example of the practicing of this invention in which the present binder constitutes the sole binder material of the molding composition, a molding composition comprising 75

40% by weight of a binder material derived from the non-cellulosic portion of woody fibrous material and 60% by weight of wood flour was molded at a temperature of 177° C. and a pressure 5 of 1100 lbs. per square inch. It was found to have the desired low water absorption, solvent resisting, etc., properties above described. In 10 appearance the surface of the molded article was a bright shiny black, changing to a brown finish only after extended exposure to water.

As an example showing the use of the binder in conjunction with mineral filler materials, the molding composition comprised 28% by weight of a binder derived from the non-cellulosic portion 15 of woody fibrous material, 35% by weight of barytes, 35% of rotten stone, and 2% by weight of gum copal, forming a molding compound having thermoplastic characteristics, and producing a very hard surfaced material.

20 As another example of the carrying out of the invention, a mixture of suitable proportions of binder and filler was placed in a cold mold and the mold brought up to temperature under pressure. Somewhat improved results as regards uniformity and low water absorption were obtained 25 by this process, the binder and the filler being in contact for a longer period of time permitting more thorough intermixture and impregnation of the filler by the binder.

30 The binder is also usable in conjunction with or in substitution for other binder materials to provide for obtaining a desired effect when the molding material is subjected to heat and pressure. Thus when used alone as the binder, or when used 35 with other binders having thermoplastic properties, the molded product is of thermoplastic character. However, the binder material of this invention may also be used in conjunction with a binder having thermosetting characteristics, such 40 as phenol-formaldehyde resin, to provide a thermosetting molded product. When the thermosetting binder is present in amounts of 50% or more by weight of the total binder, the remainder comprising the binder of this invention, such thermosetting binder exercises a dominant effect upon 45 the product and the molded product has desirable thermosetting properties. And by reason of a substantial quantity of the material of this invention, the product is produced less expensively.

50 Thus for instance a thermosetting material may be provided comprising 50% to 60% of a suitable filler, and 50% to 40% binder of which 50% or more comprises a thermosetting binder material such as phenol-formaldehyde resin, and up to 55 50% comprises the binder derived from the non-cellulosic portion of woody fibrous material. The thermosetting material of the above composition is found to be practically unaffected by boiling water and has a resistance to solvents comparable 60 with that of the ordinary molded materials in which the binder consists entirely of phenol-formaldehyde resins and the like.

As in the case of the thermoplastic compound, the thermosetting compound can be molded over 65 a wide range of temperatures and pressures but preferably the molding conditions are made approximately those now standard practice in the art. For instance, with a mixture comprising by weight 50% wood flour, 35% phenol-formaldehyde resin, and 15% of binder derived from the non-cellulosic portion of woody fibrous material (30% of the binder being such non-cellulosic portion of woody fibrous material), the mixture has been satisfactorily molded at a temperature of 70 180° C. and a pressure of 1900 lbs. per square inch,

the molding time being 1½ minutes. The materials are mixed in any desired manner, such as by grinding or milling, and a cold molded pill is made. The pill is then introduced into the mold, which has been heated to the desired temperature, and the pressure is applied, the pressure being maintained for a predetermined time and then released without cooling. The molded product has good strength, low water absorption, so that it is resistant even to boiling water, is resistant to acids and ordinary solvents, and is thermosetting.

The present invention therefore provides a binder material available in large quantities and at low cost, which can be used very satisfactorily 15 with a filler either alone or in conjunction with other known binder materials in molding compounds, either to produce a thermoplastic compound, or when used in conjunction with a binder having thermosetting properties, to produce such 20 thermosetting molding compound. Furthermore no material departure from standard molding practice or apparatus is required.

While the processes and products herein described constitute preferred embodiments of the 25 invention, it is to be understood that the invention is not limited to these precise processes and products, and that changes may be made therein without departing from the scope of the invention which is defined in the appended claims.

What is claimed is:

1. The method in the treatment of black liquor from the paper pulping industry, and the like, to recover therefrom a lignin derivative material which comprises subjecting such liquor substantially in its initial condition to a neutralizing action by passing a carbon dioxide containing gas therethrough, carrying such neutralizing forward to a controlled pH value of approximately pH 7.8 to pH 9 to precipitate from the black liquor a separated fraction of said lignin material constituting a fraction up to approximately 25% of the total solids in such liquor, separating and washing the precipitated lignin, and adding a strong acid to said precipitated lignin material while approximately at room temperature in an amount substantially that required for neutralization.

2. The method in the treatment of black liquor from the paper pulping industry, and the like, to recover therefrom a lignin derivative material which comprises subjecting such liquor substantially in its initial condition to a neutralizing action by passing a carbon dioxide containing gas therethrough, carrying such neutralizing forward to a controlled pH value of approximately pH 7.8 to pH 9 to precipitate from the black liquor a separated fraction of said lignin material constituting a fraction up to approximately 25% of the total solids in such liquor, separating and washing the precipitated lignin, and adding a strong acid to said precipitated lignin material in an amount substantially that required for neutralization and for breaking down of organo-metallic compounds.

3. The method in the treatment of black liquor from the paper pulping industry, and the like, to recover therefrom a lignin derivative material which comprises subjecting such liquor substantially in its initial condition to a neutralizing action by passing a carbon dioxide containing gas therethrough, carrying such neutralizing forward to a controlled pH value of approximately pH 7.8 to pH 9 to precipitate from the black liquor a separated fraction of said lignin material constituting a fraction up to approximately 25% of the total solids in such liquor, heating said sus-

- ension to a temperature of approximately 50° C. to 90° C. to cause coagulation and agglomeration of the precipitated particles while avoiding formation of a gummy mass thereof, separating and 5 washing the precipitated lignin material, and adding a strong acid to said precipitated lignin material in an amount substantially that required for neutralization and for breaking down of organo-metallic compounds.
- 10 4. The method in the treatment of black liquor from the paper pulping industry, and the like, to recover therefrom a lignin derivative material which comprises subjecting such liquor substantially in its initial condition to a neutralizing action by passing a carbon dioxide containing gas therethrough, carrying such neutralizing forward to a controlled pH value of not in excess of approximately pH 8.5 and within a range to precipitate from the black liquor a separated fraction 5 of said lignin material constituting a fraction up to approximately 25% of the total solids in such liquor, separating and washing the precipitated lignin, and adding a strong acid to said precipitated lignin material in an amount substantially 10 that required for neutralization and for breaking down of organo-metallic compounds.

HERMAN J. REBOULET.